

## UNITED STATES PATENT OFFICE

2,482,546

## PHENOXYALKYLAMINES AS ACCELERATORS FOR PHOTOGRAPHIC DEVELOPERS

Frank J. Kaszuba, Binghamton, N. Y., assignor to  
General Aniline & Film Corporation, New  
York, N. Y., a corporation of Delaware

No Drawing. Application July 9, 1948,  
Serial No. 37,965

12 Claims. (Cl. 95—88)

1

This invention relates to photographic developers and particularly to phenoxyalkylamines as accelerators for photographic developers.

It is well known that various amines, such as primary and secondary alkyl and alkylene amines containing from 3 to 7 carbon atoms, and heterocyclic amines such as morpholine and piperidine as disclosed in United States Patent No. 2,304,025, may be added to photographic black and white and color developing solutions for the purpose of increasing the rate of development. In other words, these amines accelerate the development so as to cause the developing agent to form the image (silver or color image) more rapidly than is possible without the presence of such amines.

Although developing solutions containing such amines cut the developing time to 12-15 minutes, such period is still unsatisfactory where large scale operations are involved, as in commercial processing where time is of the essence.

It is also known that there are aralkylamines which, when present in developing solutions in an amount ranging from 8 to 30 cc. per liter, energize weak developers to the extent that second exposure is not necessary for reversal development. It has always been assumed by the art, however, that all of these amines, in order to be operative as energizers for developing solutions, must be free from groups, such as nitro, hydroxy, sulfonic acid, halogen atoms, e. g., chlorine, bromine, and the like. Moreover, most amines are somewhat toxic and lead to skin eruptions when development of the film is done with bare hands.

I have found that phenoxyalkylamines greatly accelerate development rates and energize weak developers to an extent that no second exposure is necessary for reversal development, even if they contain a nitro group or a halogen in the aryl ring. Such phenoxyalkylamines, moreover, are less toxic than the aralkylamines of the prior art which are substituted or unsubstituted in the aryl ring by a negative group.

It is, therefore, an object of the present invention to provide a black and white and color developer having an increased rate of development so that the developing time is substantially decreased to about one-half of the normal time, and which developer is less toxic than those heretofore used.

Other objects will appear hereinafter.

The phenoxyalkylamines employed in accordance with the present invention are represented by the following general formulae:

5 and

10



wherein R and R<sub>1</sub> are hydrogen or methyl, R being hydrogen when R<sub>1</sub> is methyl and vice versa, n is a positive integer of from 2 to 3, and X is hydrogen, a nitro group, or a halogen such as chlorine, bromine and the like.

The following are examples of such phenoxyalkylamines:

20

 $\beta$ -Phenoxyethylamine

25

 $\gamma$ -Phenoxypropylamine

30

 $\beta$ -Phenoxy- $\alpha$ -methylethylamine

35

 $\beta$ -Phenoxypropylamine

40

 $\beta$ -(4-bromophenoxy)-ethylamine

45

 $\beta$ -(4-nitrophenoxy)-ethylamine

55

 $\gamma$ -(4-chlorophenoxy)-propylamine

The foregoing amines are prepared according to the methods described in Ber. 22, 3256 (1889), Ber. 24, 189 (1891), and Ber. 70B, 985 (1937).

These amines possess limited solubility in water and in alkaline developers. Their solubility in water and in alkaline developers, however, is made appreciable by converting the base into a salt such as, for example, the sulfate, hydrochloride, or carbonate. The sulfate and hydrochloride salts are readily prepared by the addition of a stoichiometrical quantity of dilute sulfuric acid and hydrochloric acid, respectively, and the carbonate is prepared by bubbling CO<sub>2</sub> into an alcohol, ether, or benzene solution of the base.

In developing color images in multi-color photographic layers containing color formers fast to diffusion with a color developer containing a phenoxyalkylamine, the developing time is cut from 20-30 minutes to 2-10 minutes. All of the layers are simultaneously developed, and the dye images formed are of excellent quality.

The developing time with black and white developers, for instance, solutions of hydroquinone and p-monomethylaminophenol sulfate and the like, is also cut to about one-half without causing fog when such solutions contain a phenoxyalkylamine.

The most useful concentrations in black and white and color developers range from about 1 to 8 grams per liter of developer solution.

As illustrative developing solutions containing such phenoxyalkylamines, the following are given:

#### Example I

|                                 |       |      |
|---------------------------------|-------|------|
| p-Monomethylaminophenol sulfate | grams | 0.08 |
| Sodium sulfite (anhydrous)      | do    | 45   |
| Hydroquinone                    | do    | 1.2  |
| Sodium carbonate (monohydrate)  | do    | 8    |
| Potassium metabisulfite         | do    | 4    |
| Potassium bromide               | do    | 1.5  |
| β-Phenoxyethylamine             | do    | 4    |
| Water to make                   | liter | 1    |

This tank developer gives, on development at 20° C. of the usual roll film, a negative in about 6 to 8 minutes after fixing and washing. The time required to develop a similar roll in the same developer and at the same temperature, but containing no β-phenoxyethylamine, ranges from 15 to 20 minutes. Increasing the concentration of the β-phenoxyethylamine to 6 grams per liter effects a further decrease in time.

#### Example II

The following developer requires 30 minutes at 20° C. to give a satisfactory degree of color development with color paper:

|                                            |       |       |
|--------------------------------------------|-------|-------|
| Sodium hexametaphosphate                   | grams | 1.0   |
| Sodium bisulfite                           | do    | 2.0   |
| p-Amino di(β-hydroxyethyl) aniline sulfate | do    | 6.3   |
| Sodium carbonate                           | do    | 100.0 |
| Hydroxylamine hydrochloride                | do    | 1.0   |
| Potassium bromide                          | do    | 1.0   |
| Water to make                              | liter | 1     |

By the addition of 5 grams of β-(4-bromophenoxy)-ethylamine to the foregoing developing solution, a color paper of excellent color rendition is developed in about 8 minutes. Increasing the concentration of the amine further reduces the time of development.

The color photographic multi-layer element

utilized in the foregoing example, consists of an integral tri-pack emulsion coated on either the usual paper base, or a clear cellulose acetate or nitrate film base, or in some cases an opaque white film base. Each of the emulsion layers is sensitized to one of the primary colors of light, namely, blue, green, and red. The top layer is blue sensitive. A filter layer, yellow in color and blue absorbing, lies under the top layer. Below this filter layer, lies a green sensitive emulsion layer, and below this a red sensitive emulsion layer. Each of the three silver-halide emulsion layers contains dye forming compounds which unite during the development of a silver image in

an aromatic amine developing agent to form a dye with the oxidation product of the developing agent. As silver is also formed during development, it must be removed after color development by treatment in a bleach, followed by a bath of sodium thiosulfate, as is well known to the art. A yellow dye is formed in the blue sensitive emulsion; a magenta dye is formed in the green sensitive emulsion; and a cyan dye is formed in the red sensitive emulsion. The combination of the dye images from these three printing primaries yields the color picture. Suitable methods for the preparation of multi-color emulsion layers have been described in the literature relating to color photography, and are, therefore, 30 not described here.

#### Example III

The following developer requires 19 minutes at 20° C. to give a satisfactory degree of color development with color paper:

|                                          |       |     |
|------------------------------------------|-------|-----|
| Sodium hexametaphosphate                 | grams | 1.0 |
| Sodium bisulfite                         | do    | 2.0 |
| 4-amino-ethylhydroxyethylaniline sulfate | do    | 6.7 |
| Sodium carbonate                         | do    | 100 |
| Hydroxylamine hydrochloride              | do    | 1.0 |
| Potassium bromide                        | do    | 1.0 |
| Water to make                            | liter | 1   |

By the addition of 4 grams of β-(4-chlorophenoxy)-propylamine to the foregoing developing solution, a color paper of excellent color rendition is developed in about 8 minutes. Increasing the concentration of the amine to 6 grams reduces the time of development to 6 minutes with the same results.

#### Example IV

The color developer of the preceding example with the addition of 5 grams of β-phenoxyethylamine developed a multi-layer color film sheet, of the reversal type, and containing color formers fast to diffusion, in about 8 minutes at 20° C., whereas without the β-phenoxyethylamine, the time required to color develop the said film sheet is over 30 minutes.

The above examples are to be regarded as merely illustrative of the invention and not in any sense restrictive. It will be obvious to those skilled in the art that many modifications, such as substituting equivalent materials and varying the proportions of the materials used are within the spirit and scope of the invention. The scope, therefore, of the invention is to be limited solely by the following claims.

I claim:

1. An alkaline photographic developer for silver-halide emulsions comprising an aromatic silver-halide developing agent and a phenoxy-

5

alkylamine selected from the class consisting of those corresponding to the following formulae:



5

6

exposed silver-halide emulsion in an alkaline developer containing an aromatic silver-halide developing agent for said emulsion and a developing accelerator characterized by the formula:



and



5

10

wherein R and R1 represent a group selected from the class consisting of hydrogen and methyl, R being hydrogen when R1 is methyl and R1 being hydrogen when R is methyl, n is a positive integer of from 2 to 3, and X is a group selected from the class consisting of hydrogen, nitro and halogen, and the salts of said amines.

2. An alkaline photographic developer for silver-halide emulsions comprising an aromatic silver-halide developing agent and a phenoxyalkylamine characterized by the following formula:



20

3. An alkaline photographic developer for silver-halide emulsions comprising an aromatic silver-halide developing agent and a phenoxyalkylamine characterized by the following formula:



30

4. An alkaline photographic developer for silver-halide emulsions comprising an aromatic silver-halide developing agent and a phenoxyalkylamine characterized by the following formula:



40

5. In the development of a photographic negative, the step comprising the development of an exposed silver-halide emulsion in an alkaline developer containing an aromatic silver-halide developing agent for said emulsion and a developing accelerator selected from the class consisting of phenoxyalkylamines corresponding to the following formulae:



50

and



45

60

wherein R and R1 represent a group selected from the class consisting of hydrogen and methyl, R being hydrogen when R1 is methyl and R1 being hydrogen when R is methyl, n is a positive integer of from 2 to 3, and X is a group selected from the class consisting of hydrogen, nitro and halogen, and the salts of said amines.

6. In the development of a photographic negative, the step comprising the development of an

65

exposed silver-halide emulsion in an alkaline developer containing an aromatic silver-halide developing agent for said emulsion and a developing accelerator characterized by the formula:



70

75

7. In the development of a photographic negative, the step comprising the development of an exposed silver-halide emulsion in an alkaline developer containing an aromatic silver-halide developing agent for said emulsion and a developing accelerator characterized by the formula:



25

8. In the development of a photographic negative, the step comprising the development of an exposed silver-halide emulsion in an alkaline developer containing an aromatic silver-halide developing agent for said emulsion and a developing accelerator characterized by the formula:



35

9. A color-forming photographic developer comprising a primary aromatic amino developing agent and a phenoxyalkylamine selected from the class consisting of those corresponding to the following formulae:



and



45

60

wherein R and R1 represent a group selected from the class consisting of hydrogen and methyl, R being hydrogen when R1 is methyl and R1 being hydrogen when R is methyl, n is a positive integer of from 2 to 3, and X is a group selected from the class consisting of hydrogen, nitro and halogen, and the salts of said amines.

10. A color-forming photographic developer comprising a primary aromatic amino developing agent and a phenoxyalkylamine characterized by the following formula:



65

11. A color-forming photographic developer comprising a primary aromatic amino developing agent and a phenoxyalkylamine characterized by the following formula:



70

75

12. A color-forming photographic developer

comprising a primary aromatic amino developing agent and a phenoxyalkylamine characterized by the following formula:



FRANK J. KASZUBA.

#### REFERENCES CITED

The following references are of record in the file of this patent:

5. UNITED STATES PATENTS

| Number       | Name             | Date          |
|--------------|------------------|---------------|
| 2,181,941    | Goldacker et al. | Dec. 5, 1939  |
| 2,327,813    | Nadeau et al.    | Aug. 24, 1943 |
| 10 2,371,740 | Dearing et al.   | Mar. 20, 1945 |